

## UNITED STATES PATENT OFFICE

2,370,898

PRODUCTION OF METALLIC MAGNESIUM BY  
FERROSILICON REDUCTION

Leslie Victor Whiton and Hugh McLaurin Weld,  
Haley, Ontario, Canada, assignors to Dominion  
Magnesium Limited, Toronto, Ontario, Canada,  
a corporation of the Province of Ontario

No Drawing. Application October 27, 1943, Serial  
No. 507,882. In Canada October 18, 1943

5 Claims. (Cl. 75—67)

This invention relates to the production of metallic magnesium by thermal reduction of magnesia-containing materials with ferrosilicon, and is particularly directed to an improvement in the procedure set forth in L. M. Pidgeon Canadian Patents Nos. 415,764 and 415,765, issued October 12, 1943.

As disclosed in these patents magnesia-containing material and ferrosilicon, in the form of briquettes, are heated under reduced pressure in externally fired metal retorts, horizontally disposed within a furnace, to reduce the magnesia, volatilize the magnesium and condense the latter in dense coherent structural form. The vapours evolved from the charge are condensed in a portion of each retort extending outside the furnace and within which is located removable condenser sleeve for removal with the condensed magnesium. Means may be provided for the condensation and independent removal of metals having a higher vapour pressure than magnesium. While the retorts remain within the furnace under operating temperatures of 1100 to 1200° C. the condenser end of each retort is opened to the air for removal of the condensed metal, discharge of the residue and recharging. The retorts may be 6 to 12 inches in diameter, preferably 8 or 10 inches, and are charged and discharged in groups in an operating cycle which may vary from say 6 to 12 hours.

During the operating cycle the hot retorts are charged with briquettes, evacuated to remove steam, occluded and adsorbed gases and the charge is maintained under a very low pressure of say 0.02 mm. Silicon vapour is evolved from the ferrosilicon and this vapour reduces the magnesia to magnesium which is volatilized and condensed. At the end of the cycle when the magnesium has been volatilized and condensed the exposed ends of the retorts are opened to the air and discharged.

It is known that the reaction proceeds best when lime is present with the magnesia. The theoretical equation representing the reaction is as follows:



That is to say, one molecular weight of silicon, derived from the ferrosilicon, liberates as vapour two molecular weights of magnesium. The theoretical ratio of calcine ( $\text{MgO} \cdot \text{CaO}$ ) to silicon in the charge is 1 to 0.146. When 75% ferrosilicon is used 0.194 pound is required to provide 0.146 pound of silicon and the theoretical ratio of calcine to ferrosilicon is 1 to 0.194. In practice

a ratio of calcine to silicon of 1 to 0.132, that is an excess of calcine, as well as the theoretical ratio have been used.

An object of the present invention is to improve the overall economic efficiency of this method. A more specific object is to obtain a maximum recovery of magnesium in the calcine during its passage through the operating cycle. A further object is to increase the efficiency of the ferrosilicon used and to reduce the amount of heat required per pound of magnesium recovered.

It has been found that greatly improved results are obtained by using 110 to 130% of the theoretical amount of silicon required for the reaction. The invention thus contemplates using a ratio of calcine to silicon within the range of 1 to 0.160 and 1 to 0.189. Best results have been obtained by using 115% of the theoretical amount of silicon, that is a ratio of calcine to silicon of 1 to 0.167.

It is known that commercial ferrosilicon may contain varying amounts of silicon and due regard must be given to the actual silicon content of the ferrosilicon used when determining the amount to be employed in providing the desired ratio of calcine to silicon.

It appears that the increased concentration of ferrosilicon in the briquettes charged into the retorts causes a more rapid transfer of heat into and throughout the charge. Thus in a given period of time the charge absorbs a greater amount of heat and the temperature more quickly reaches the effective reaction point. Also with the greater concentration of ferrosilicon the concentration of silicon vapour is increased to cause the reaction to go forward to more completely reduce the magnesia and liberate the metal.

To illustrate the improvements effected by the invention the following examples are given.

Calced dolomite was mixed with ferrosilicon in proportions to provide 115% of the theoretical amount of silicon required and the mixture was briquetted in the usual manner and charged into the hot retorts. The ratio of calcine to silicon was 1 to 0.167. In an eight hour operating cycle the increase in the amount of magnesium recovered from the charge was 26.3%, as compared with the former practice in which a ratio of calcine to silicon of 1 to 0.132 was used.

Using a ratio of calcine to silicon of 1 to 0.167 in an operating cycle of 10 hours the amount of magnesium recovered was increased by 37.5% as compared with the former practice. That is to say, the amount of silicon required per pound

of magnesium recovered was only 91.9% of that previously used. At the same time the heat requirements of the furnace per pound of magnesium recovered was reduced by about 20%.

Moreover the structures, or so-called crowns, of magnesium formed in the condenser are heavier and more compact with greater mechanical strength. As a result fewer fines are produced in handling the crowns. Accordingly, there is a reduction in melting loss and in flux consumption in melting the crowns and casting the metal into ingots.

We claim:

1. In the production of magnesium by thermal reduction of magnesia-containing material with ferrosilicon the step which comprises heating in a retort under reducing conditions briquettes comprising the magnesia-containing material and ferrosilicon in proportions to provide 110 to 130% of the theoretical amount of silicon for the reaction.

2. A method as defined in claim 1 wherein calcined dolomite is mixed with ferrosilicon in proportions to provide at least 10 and not more than 30% of silicon in excess of the theoretical amount required for the reaction.

3. A method of producing metallic magnesium which comprises calcining dolomite, and heating under reducing conditions the calcined dolomite with ferrosilicon in proportions to provide a ratio of calcine to silicon between 1 to 0.160 and 1 to 0.189.

4. A method of recovering magnesium from magnesia-containing material which comprises the step of heating under reducing conditions the magnesia-containing material with ferrosilicon in proportions to provide substantially 15% silicon in excess of the theoretical amount required for the reaction.

5. A method of recovering magnesium from magnesia-containing material by thermal reduction which comprises heating under reducing conditions said material containing one mole of magnesia per mole of lime with ferrosilicon in proportions to provide 10 to 30% silicon in excess of the theoretical amount required for the reaction.

LESLIE VICTOR WHITON.  
HUGH McLAURIN WELD.